

# UNITED STATES PATENT OFFICE.

SILAS R. DIVINE, OF LOCH SHELDRAKE, NEW YORK, ASSIGNOR TO THE  
REND ROCK POWDER COMPANY, OF NEW JERSEY.

## EXPLOSIVE COMPOUND.

SPECIFICATION forming part of Letters Patent No. 289,756, dated December 4, 1883.

Application filed July 23, 1883. (No specimens.)

*To all whom it may concern:*

Be it known that I, SILAS R. DIVINE, of  
Loch Sheldrake, Sullivan county, State of New  
York, and a citizen of the United States, have  
5 invented an Improved Explosive Compound,  
of which the following is a full, clear, and ex-  
act description.

The object of my invention is to provide an  
explosive compound for blasting and other  
10 purposes, the ingredients of which can be  
handled and transported separately without  
hazard from explosion, and can be united by  
the consumer to form the explosive at the time  
when and the place where its use is desired.

15 My invention consists of an explosive com-  
pound composed of two ingredients, the one a  
solid—such as chlorate of potash in a crushed  
or powdered state—and the other a liquid,  
such as the heavy oil of coal tar, which is  
20 commonly called "dead-oil." These ingredi-  
ents are combined to form the explosive by  
allowing the solid ingredient to absorb the  
liquid ingredient; and this can be done by the  
workman or miner at the place and when the  
25 explosive is desired for use. The theoretical  
proportions in which the said ingredients com-  
bine effectively to constitute my explosive  
compound are about seven and one-half parts  
of chlorate of potash to one part of dead-oil.  
30 The exact theoretical proportions need not,  
however, be strictly adhered to, as a variation  
somewhat therefrom will still yield an effective  
explosive.

Perchlorate or permanganate of potash may  
be employed as the solid ingredient of the 35  
compound, and other fluid hydrocarbons  
which are practically non-volatile in a free  
state at ordinary temperatures—say such as  
have a boiling-point above about 300° Fahrenheit—may be used as the liquid ingredient. 40

The ingredients of my improved explosive  
compound may, if desired, be mixed in the  
proper proportions in a convenient receptacle.

In Letters Patent No. 243,432, dated June  
28, 1883, I have described an explosive com- 45  
pound of this character composed of a solid  
ingredient—such as chlorate of potash—and a  
liquid ingredient—such as nitro-benzole, or  
other liquid nitro compound—and therefore I  
do not intend to claim herein a compound com- 50  
posed of such named ingredients.

What I claim as my invention, and desire to  
secure by Letters Patent hereunder, is—

The explosive compound herein described,  
which consists of a solid ingredient—a chlorate 55  
of potash—and a liquid ingredient—as the  
heavy oil of coal-tar (dead-oil)—mechanically  
united substantially in the proportions and as  
and for the purposes set forth.

SILAS R. DIVINE.

Witnesses:

A. S. FITCH,  
WM. T. FARNHAM.